

## UNITED STATES PATENT OFFICE

1,985,236

## PARTI-COLORED LEATHER

Peter A. Blatz, Westover Hills, Del.

No Drawing. Application January 27, 1932  
Serial No. 589,316

2 Claims. (Cl. 91—68)

My invention relates to the manufacture of parti-colored leather, and comprises an improved method of applying an insoluble parti-colored coating to the surface of a chrome or otherwise tanned hide or skin which may be subsequently glazed in a manner precisely similar to the method of glazing of ordinary kid skins.

While the application of an insoluble coating to a leather surface, such as a hide or skin, may be carried out in other ways, I have developed a method of imparting a parti-colored coating to the surface of the hide or skin that partakes of a stippled or mottled effect. In practice, a ground color of a light or pastel, or, in some instances, white shade, is applied to the surface of the skin. The ground coating is of any suitable light or white pigment dissolved in casein, and it may be brushed upon the surface of the skin, or applied by means of a pad, or in any way that will insure the application of a solid, even tone of a light or white color or shade. Upon the surface thus prepared I spatter a contrasting shade or color in dots or drops in a fairly even manner, for which purpose I may use an air brush of usual type. This spattering or stippling is applied to the skin over the entire surface of the same, preferably in a series of applications immediately succeeding each other.

Parti-colored leathers are suitable and desirable for numerous purposes and parti-colored kid or sheep skin is particularly applicable for use as a lining for the inner heel portions of shoes in a color which supplements or contrasts with the color of the leather or skin from which the shoe is made, particularly when such shoes or slippers are made from the skins of reptiles such as lizards, snakes, alligators, and/or the like. Such lining skins or leathers have heretofore been of one color, shade or tone. Due to numerous reasons, a large number of skins when colored in the usual or ordinary manner are imperfect from the coloring point of view while still suitable for many uses when the quality of the skin is considered. Similarly, many skins which cannot be colored suitably in one tone or shade, due to imperfections in the skin or for other reasons, would be highly suitable for various purposes if they could be colored or ornamented in a manner that would hide the imperfections.

One object of my invention is to provide a novel method or process of making parti-colored hides or skins.

A further object of my invention is to provide a method of parti-coloring skins in such a manner that a mottled effect may be obtained and

imperfections in the skin itself, or imperfections resulting from prior coloring operations hidden.

A more specific object of my invention is to provide a method of manufacturing parti-colored skins involving the application of two or more colors to the surface of the same, usually the grain surface, which subsequently may be glazed.

My process consists in the application to a tanned skin of various coats of different and differently colored materials and in subjecting such skins to a definite process of treatment. My process begins at the time the hides or skins are completely tanned and are ready for any suitable use, prior to the glazing step. Taking such material, which will be hereinafter referred to as "skins", which may be chrome or otherwise tanned, the first step in my process is to whiten or light coat one or both surfaces of the skin with a suitable white or light pigment carried by or in solution in a casein medium. If desired, pigments other than white may be used and the base coat may be a suitable dye and not necessarily a pigment dissolved in a casein base.

A coating of this material may be spread over one or both sides of the skin in any suitable manner as by the use of a brush, pad, swab or the like, and such color may then be leveled, i. e., brought to a single tonal effect, by the further application of a solution of the pigment of the desired tone, by means of an air brush. Optionally, the skin may be dipped in a dye vat. I thus form upon one or both sides of the skin a base coating or background of a single color which may be any tone or shade suitable for the purpose, preferably light, or any shade or tone demanded by the trade.

After the base coating has completely dried, the skin is subjected to a plurality of coating steps in which a contrasting color (darker on light grounds and lighter on dark grounds) is applied to the ground color or shade. This second coating application, which is the first coating designed to produce the mottled effect, is preferably applied with an air brush or spray gun, in such manner that the contrasting color appears upon the base or ground coat as a mass of fine dots or spots of relatively minute size which may range from that of a pin point up to  $\frac{1}{2}$ " in diameter. The pigment of the contrasting color coating thus applied, similarly to that of the base or ground coat, should be carried by or dissolved in a casein medium, but, under some circumstances and for some conditions it may be a dye, or other coloring material.

Immediately upon the completion of the appli-

cation of one such stippled or dotted coating to the entire surface of the skin operated upon, a second similar stippled or dotted coating is applied, followed by as many as three or four other 5 coating applications depending upon the amount of covering desired. In all instances a plurality of stippled or dotted coatings are applied. Each of these coatings should be successively applied over the entire surface of the skin and before 10 the preceding coating is entirely dry; my practice being to start at one point of the skin; the upper left hand corner, for instance, and as soon as one coating has been applied, to start the second from the same point, and so on until the 15 final coating has been applied. The dots or spots of the successive coating applications tend to run together quite promiscuously over the coated surface and this tendency of the dots or spots to run together, governed by the consistency of the 20 coating body, its drying speed, the speed of its application, etc., determines the number of dotted or stippled coatings to be applied. In practice it is desirable to only apply sufficient coatings to cause the dots to partially run together in anything 25 but a regular manner and always in a way that will allow the base to partially be seen or 30 grin through the dotted surface; the dotted coatings thus applied creating a mottled effect. If too many stippled or dotted coatings are applied, of course, the skin will have a complete covering of the contrasting color and the base or ground coat will not appear.

Upon completing the application to the skins of the last dotted coating of the contrasting coloring material, the skin is allowed to dry. After 35 the skins are completely dry they may be glazed in the usual manner. As a final step, they may be made perfectly flat by pressure between the

heated plates of a hydraulic press or in any other suitable and satisfactory manner.

Various modifications may be made in the above-described embodiment of my invention without departing from the spirit and scope 5 thereof as set forth in the following claims.

I claim:

1. The method of making parti-colored skins which comprises completely tanning the skin to produce leather, applying to the entire surface 10 of such completely tanned skin a base coat of a casein-held pigment, allowing said base coat to thoroughly dry, spattering a plurality of coats of a colored pigment contrasting with the color of the base pigment in a multiplicity of spots or 15 dots over the entire surface of the base coat whereby the base coat shows through the subsequent spattering coats in a plurality of places and presents a mottled appearance, allowing the spattered coats to dry, glazing the colored surface 20 of the skin, and thereafter subjecting the mottled skin to pressure between hot plates.

2. The method of making parti-colored skins which comprises completely tanning the skin to produce leather, applying to the entire surface 25 of such completely tanned skin a base coat of a casein-held pigment light in color, allowing said base coat to thoroughly dry, spattering a plurality of coats of a dark colored pigment over the light base in a multiplicity of spots or dots 30 over the entire surface of the base coat whereby the latter shows through the subsequent spattering coats in a plurality of places and presents a mottled appearance, allowing the spattered coats to dry, glazing the colored surface of the 35 skin, and thereafter subjecting the mottled skin to pressure between hot plates.

PETER A. BLATZ.